

## UNITED STATES PATENT OFFICE

2,378,204

## MANDELIC ACID ANTIFOGGANTS

George E. Fallesen, Rochester, N. Y., assignor to  
Eastman Kodak Company, Rochester, N. Y., a  
corporation of New Jersey

No Drawing. Application January 13, 1944,  
Serial No. 518,124

5 Claims. (Cl. 95—88)

This invention relates to fog inhibitors for photographic emulsions and to photographic emulsions containing them.

It is known that photographic emulsions, particularly ultra-sensitive emulsions, or those containing color sensitizers, exhibit a tendency to form a deposit of silver in the unexposed emulsion. This deposit extends more or less uniformly over the entire emulsion and is known as fog. Photographic fog is of two types, local and general. Local fog is formed by exposure of the film or plate at undesired points, as by a light leak in the camera, or by local action of chemicals. General fog or, as it is sometimes known, chemical fog, is formed in a number of ways. It may be caused by the conditions under which the film or plate is stored, such as conditions of high temperature or unusually long time of storage. The nature of the emulsion may also produce chemical fog, as well as the conditions of development of the emulsion, as by development for protracted periods of time or at temperatures above normal. Highly sensitive emulsions are more likely to fog than those of lower sensitivity. I am concerned primarily with general or chemical fog.

It is an object of the present invention to provide antifogging or fog inhibiting agents for ultra-sensitive photographic emulsions and thereby to preserve the emulsion against deterioration resulting in fog. A further object is to provide antifogging agents which do not markedly lower the sensitivity of the emulsion. Other objects will appear from the following description of my invention.

These objects are accomplished by developing an exposed silver halide emulsion in the presence of an alkali-metal salt of a dl-mandelic acid, such as the sodium salt, preferably by incorporating the mandelic acid salt in the emulsion.

dl-Mandelic acid,  $C_6H_5CHOHCOOH$ , may be prepared from benzaldehyde and hydrocyanic acid to form benzaldehyde cyanhydrin which is then treated with hydrochloric acid to form the dl-mandelic acid. I prefer to use the sodium salt of dl-mandelic acid as an anti-fogant in emulsions although other alkali-metal salts such as the potassium or ammonium salts may be employed.

These compounds may be incorporated in an

emulsion, particularly a fast negative emulsion to which may be added optical sensitizing dyes. The emulsion may be one which is intended to be used directly after emulsification or one which is subjected to ripening.

The antifogging properties of the dl-mandelic acid salts were tested as follows:

Silver iodobromide was precipitated in 0.8% gelatin solution. After precipitation was complete, the entire volume of emulsion was cooled and divided into portions weighing 1643 grams each. To each portion was added enough gelatin to increase the gelatin concentration to approximately 6.6%. Each portion was then heated to the required digestion temperature, that is, about 60° C. and as soon as this temperature was reached a certain amount of the compound to be tested was added to it. For example, 25 grams of dl-mandelic acid was dissolved in 300 cc. of methyl alcohol, and the sodium salt formed by adding sodium hydroxide solution. The pH of this solution was adjusted to that of the emulsion before adding it to the emulsion. Digestion was then continued for 30 minutes at the specified temperature and the emulsion was then chilled and stored in preparation for shredding and washing. One of these portions received no additions other than the required gelatin and it served as the control for all the portions originating from the same precipitation of silver halide.

After washing, each emulsion was heated to the optimum point for maximum speed and gamma with acceptable fog. Unsensitized and panchromatized samples of each emulsion so finished were coated by machine on glass plates. After the plates were dry, a series of sensitometric tests were made on them. The data were then compared with those of the check emulsion containing no addendum. These tests include initial tests for speed, gamma and fog, made on the day after coating, similar tests on a second set of plates incubated at 120° F., dry heat, for 6 days and a third set of tests made on a third set of plates after having been kept under tropical conditions for 14 days. (The "tropical conditions" are simulated by varying the temperature and humidity through a cycle to reproduce day and night conditions in tropical climates.) Plates for each of these tests were developed for

3 minutes at 65° F. in Kodak D-19 developer which had the following composition:

|                                  |       |     |
|----------------------------------|-------|-----|
| Monomethyl-p-aminophenol sulfate | grams | 2.2 |
| Sodium sulfite (desiccated)      | do    | 96  |
| Hydroquinone                     | do    | 8.8 |
| Sodium carbonate (desiccated)    | do    | 48  |
| Potassium bromide                | do    | 5   |
| Water to                         | liter | 1   |

The results of these tests are tabulated below: 10

| Amount               | Initial fog tests      |                           | Tropical condition 14-day incubation fog tests |                           | 6 day 120° F. dry incubation fog tests |                           |
|----------------------|------------------------|---------------------------|------------------------------------------------|---------------------------|----------------------------------------|---------------------------|
|                      | Emulsion with compound | Emulsion without compound | Emulsion with compound                         | Emulsion without compound | Emulsion with compound                 | Emulsion without compound |
| 1.5 grams per liter  | .06                    | .06                       | .06                                            | .10                       | .07                                    | .10                       |
| 3 grams per liter    | .05                    | .06                       | .04                                            | .10                       | .08                                    | .10                       |
| 6.8 grams per liter  | .05                    | .06                       | .07                                            | .10                       | .07                                    | .10                       |
| 13.5 grams per liter | .06                    | .06                       | .05                                            | .10                       | .07                                    | .10                       |

The amount of fog was determined by reading the density at the toe of the curve after exposure and development of the emulsion, in the usual manner.

The amount of the fog inhibiting agent used in the emulsion will depend upon the composition of the agent and upon the type of emulsion. In general, the amount of fog inhibiting agent used will vary from 1 gram to 15 grams per 1000 cc. of wet emulsion. It will be understood that more or less than this amount may be used. Generally, however, if a greater amount is used in the emulsion, either no increased fog inhibiting effect is obtained or there is a decrease in the sensitivity of the emulsion. These compounds may be incorporated by mixing them with any suitable solvent which is inert with respect to the emulsion such as water, methyl alcohol, ethyl alcohol, acetone and others.

The fog inhibiting agents which I have described may be used in various kinds of photographic emulsions. In addition to being useful in ordinary non-sensitized emulsions, they may be used in orthochromatic, panchromatic and X-ray emulsions. Various silver salts may be used as the sensitive salt such as silver bromide, silver chloride, silver bromoiodide, and silver

chlorobromide. The dispersing agent may be gelatin or other suitable colloids such as collodion, albumen, cellulose organic derivatives or synthetic resins.

In addition to their use in the sensitive emulsion itself, my fog inhibiting agents may also be incorporated in the developing solution or in an overcoating or intermediate layer in the photographic element containing the sensitive emulsion layer.

It is to be understood that I contemplate as included within my invention all modifications and equivalents falling within the scope of the appended claims.

I claim:

1. A gelatino-silver halide emulsion containing a fog-inhibiting amount of an alkali metal salt of dl-mandelic acid.

2. A gelatino-silver halide emulsion containing a fog-inhibiting amount of the sodium salt of dl-mandelic acid.

3. A gelatino-silver halide emulsion containing from 1 to 15 grams per liter of wet emulsion of the sodium salt of dl-mandelic acid.

4. The method of reducing the amount of fog produced upon development of a silver halide emulsion, which comprises developing said emulsion in the presence of a fog-inhibiting amount of an alkali metal salt of dl-mandelic acid.

5. The method of reducing the amount of fog produced upon development of a silver halide emulsion, which comprises developing said emulsion in the presence of a fog-inhibiting amount of the sodium salt of dl-mandelic acid.

GEORGE E. FALLESEN.